

# United States Patent Office

2,950,992

Patented Aug. 30, 1960

1

2,950,992

## CELLOPHANE COATING HAVING IMPROVED WET STRETCH AT LOW TEMPERATURES

William O. Brillhart, LeRoy Gallant, and James N. Carver, Fredericksburg, Va., assignors to American Viscose Corporation, Philadelphia, Pa., a corporation of Delaware

No Drawing. Filed Aug. 12, 1957, Ser. No. 677,791

10 Claims. (Cl. 117—144)

This invention is directed to an improved cellophane coating. More specifically it is directed to an improved plasticizer for the conventional nitrocellulose coatings used on cellophane.

A substantial amount of cellophane production is used in packaging fresh red meat for super-market display. The cellophane intended for this purpose is coated only on one side and when it is wrapped on meat the cellophane is stretched tight and sealed in place. When the meat juices wet the inner surface of the wrapper they cause it to swell. If the cellophane coating does not have a high degree of stretch it will crack and split and the meat will blacken and discolor in those areas as a result of dehydration. The nitrocellulose coatings usually employed on cellophane do not always have the desired degree of wet stretch required for this purpose. Hence the object of this invention is to provide an improved cellophane coating having a high wet stretch at temperatures in the range of 0—5° C., since red meat is usually stored under these conditions.

We have found that acetyl tributyl citrate, when used as the major component of the plasticizer for a conventional nitrocellulose coating, will produce lacquers having a high degree of wet stretch at low temperatures. Acetyl tributyl citrate is a water white, high boiling liquid which is soluble in most common organic solvents. It is insoluble in water and resistant to hydrolysis. Toxicity studies have shown this ester may be considered essentially non-toxic. It is compatible with most natural and synthetic resins. The use of acetyl tributyl citrate as a nitrocellulose plasticizer per se is described at some length in an article entitled "Citric Acid Ester Plasticizers," by Prescott and Cragwell, Modern Plastics, October 1952, page 134. However, so far as known this ester has not been employed in a nitrocellulose coating especially designed for use on a cellophane wrapper which requires a high wet stretch at low temperatures.

A typical formula for a nitrocellulose coating composition is as follows:

|                                              | Parts |
|----------------------------------------------|-------|
| Nitrocellulose                               | 50    |
| Acetyl tributyl citrate (liquid plasticizer) | 26    |
| Dicyclohexyl phthalate (solid plasticizer)   | 13    |
| Alkyd resin                                  | 5     |
| Paraffin                                     | 4     |
| Bentonite                                    | 2     |

The above formula was dissolved in a solution consisting of 420 parts ethyl acetate and 280 parts toluene and then coated on cellophane by conventional methods followed by drying to evaporate and recover the solvent. It gave a non-blocking film which was satisfactory for meat packaging and exhibited high stretch when wet under icebox conditions.

### Example I

A 10 gallon batch of nitrocellulose lacquer was prepared using the proportions recited above. An 18-inch wide roll of cellophane was given an anchor coating of

2

Accobond 3900 (a cationic melamine-formaldehyde resin) on both sides of the sheet and was then coated on the bottom surface only with the nitrocellulose lacquer at a speed of 100 feet per minute. The top surface was left uncoated or "raw." Normal oven temperatures (230° F.) and reconditioning zone temperatures (160° F. dry bulb, 145° F. wet bulb) were used. The film was wound up on a shell after passage through the coater.

Physical tests of the film showed a strong heat seal even when the coated surface was sealed to the uncoated surface. The clarity was also good. Upon immersion in ice water for one hour and stretching the film in a transverse direction, it was observed that the base film ruptured at about 90—110% elongation without prior rupture of the coating, whereas coatings prepared with only 6—8 parts of liquid plasticizer ruptured under the same test at 40—50% elongation without rupture of the base film.

Meat packaging tests confirmed the high degree of protection afforded by this coating in resisting rupture due to expansion when rewet by meat juices. They also revealed a high degree of resistance to handling, squeezing, and tumbling such as would be experienced in regular display of the meat packages in a commercial market.

The following proportions give a fair indication of the range of the various components of lacquer, in parts by weight of the total, exclusive of solvent:

|                    | Percent |
|--------------------|---------|
| Nitrocellulose     | 45—55   |
| Total plasticizers | 36—44   |
| Resin              | 0—12    |
| Paraffin           | 3—6     |
| Bentonite          | 1—3     |

Based on lacquer solids the acetyl tributyl citrate may vary from 15—44% by weight, i.e., it may constitute the entire plasticizer since there is no blocking problem here because one does not stick two coated sides together. The preferred proportion for the acetyl tributyl citrate is 20—34% by weight of the lacquer solute. For fresh meat wrapping the liquid plasticizer should be at least 1/2 the total plasticizer content in order to give sufficient wet strength. The preferred solid plasticizers for use with the citrate include Sylflex (phthalimidooethyl propionate), dicyclohexyl phthalate, and ethyl benzoyl benzoate. Preferred resins are ester gum, copal, dammar, and maleic-modified rosin esters.

The various components described above are to be considered simply as illustrative but not limiting as to the components which could be used in the nitrocellulose lacquer. The solid plasticizers which could be used with the acetyl tributyl citrate include diphenyl phthalate, ethylene glycol dibenzoate, N-ethyl p-toluene sulfonamide, cyclohexyl p-toluene sulfonamide, ethyl oxanilate, diisobutyl tartrate, sucrose octo-acetate, acetanilide, phenyl benzoate, naphthyl benzoate, glyceryl benzoate, triphenyl phosphate, camphor, etc.

Other resins in addition to those specified above would include resinate, hydrogenated rosin, hydrogenated rosin esters, kauri, alkyd resins, vinyl derivatives, chlorinated diphenyl resins, and soluble resins of the phenol-formaldehyde type.

The wax or wax-like material used in moistureproofing as moistureproofing agents include, in addition to paraffin, petrodatum, ceresin, japan wax, palm wax, beeswax, certain chlorinated hydrocarbons, Chinese insect wax, or other synthetic waxes or wax-like materials may be used. If some of these waxes are too soft for the purpose desired, they may be mixed with harder waxes of the group or with carnauba wax, candelilla wax or other harder waxes. Generally, paraffin serves as a satisfactory mois-

tureproofing agent which may be hardened, if necessary, by admixture with carnauba wax or candelilla wax.

Anchor coatings are well known and a variety of these could be used in the present application. These would include phenol formaldehyde resins, urea formaldehyde resins, melamine formaldehyde resins, polyethylene imine having a degree of polymerization above 50, etc.

Instead of the bentonite slip agent one may use talc, kaolinite,  $ZnO$ , etc.

As solvents, there may be employed any of the known lacquer solvents such as alcohols, ketones, esters, hydrocarbons, ethers, halogenated hydrocarbons, nitro paraffins, or mixtures of the foregoing solvents, etc.

Application Serial No. 677,802, filed August 12, 1957, wherein Brillhart is a co-applicant, discloses and claims the use of acetyl tributyl citrate in a nitrocellulose coating on cellophane in order to prevent ink-bleeding thereon.

We claim:

1. A sheet of regenerated cellulose carrying a coating having a high wet stretch at temperatures in the range of about 0 to 5° C., said coating comprising as its principal constituents nitrocellulose and a plasticizer composition, said plasticizer composition consisting essentially of about 36 to 44% by weight of said coating, acetyl tributyl citrate constituting one component of said plasticizer composition and being present in an amount of from about 15 to 44% by weight of said coating, the balance of said plasticizer composition being a solid plasticizer selected from the group consisting of phthalimidoethyl propionate, dicyclohexyl phthalate, ethyl benzoyl benzoate, diphenyl phthalate, ethylene glycol dibenzoate, N-ethyl p-toluene sulfonamide, cyclohexyl p-toluene sulfonamide, ethyl oxanilate, diisobutyl tartrate, sucrose octo-acetate, acetanilide, phenyl benzoate, naphthyl benzoate, glycercyl benzoate, triphenyl phosphate, and camphor.

2. The coated sheet of claim 1 wherein said acetyl tributyl citrate varies from about 20 to 34% by weight of said coating and said solid plasticizer varies from about 2 to 24% by weight of said coating.

3. The sheet of claim 2 wherein said solid plasticizer is phthalimidoethyl propionate.

4. The sheet of claim 2 wherein said solid plasticizer is dicyclohexyl phthalate.

5. The sheet of claim 2 wherein said solid plasticizer is ethyl benzoyl benzoate.

6. A method of preparing a sheet of regenerated cellulose having a coating which possesses a high wet stretch at temperatures in the range between about 0 and 5° C. comprising applying to said sheet of regenerated cellulose a lacquer containing as its principal constituents nitrocellulose and acetyl tributyl citrate as a liquid plasticizer, said lacquer exclusive of the solvent therefor comprising in percent by weight about 45 to about 55% nitrocellulose and about 36 to about 44% by weight of plasticizer, of which about 15 to 44% by weight is acetyl tributyl citrate and the balance of said plasticizer being a solid plasticizer selected from the group consisting of phthalimidoethyl propionate, dicyclohexyl phthalate, ethyl benzoyl benzoate, diphenyl phthalate, ethylene glycol dibenzoate, N-ethyl p-toluene sulfonamide, cyclohexyl p-toluene sulfonamide, ethyl oxanilate, diisobutyl tartrate, sucrose octo-acetate, acetanilide, phenyl benzoate, naphthyl benzoate, glycercyl benzoate, triphenyl phosphate, and camphor.

7. The method of claim 6 wherein said acetyl tributyl citrate varies from about 20 to about 34% by weight of said lacquer exclusive of solvent therefor and said solid plasticizer varies from about 2 to 24% by weight of said lacquer exclusive of solvent therefor.

8. The method of claim 7 wherein said solid plasticizer is phthalimidoethyl propionate.

9. The method of claim 7 wherein said solid plasticizer is dicyclohexyl phthalate.

10. The method of claim 7 wherein said solid plasticizer is ethyl benzoyl benzoate.

#### References Cited in the file of this patent

#### UNITED STATES PATENTS

|           |               |       |               |
|-----------|---------------|-------|---------------|
| 1,997,105 | Cornwell      | ----- | Apr. 9, 1935  |
| 2,000,251 | Rankin        | ----- | May 7, 1935   |
| 2,177,645 | Flint et al.  | ----- | Oct. 31, 1939 |
| 2,279,788 | Jebens        | ----- | Apr. 14, 1942 |
| 2,311,831 | Heaven et al. | ----- | Feb. 23, 1943 |
| 2,770,555 | Cornwell      | ----- | Nov. 13, 1956 |

#### FOREIGN PATENTS

|         |               |       |               |
|---------|---------------|-------|---------------|
| 753,318 | Great Britain | ----- | July 25, 1956 |
|---------|---------------|-------|---------------|

#### OTHER REFERENCES

Prescott et al.: Modern Plastics, vol. 30, 10/52, p. 134 ff.